

## 1

2,993,749

### CELLULOSE ESTERS WITH DIMENSIONAL STABILITY

William G. Sloan and Arthur M. Du Pré, Jr., New Orleans, La., Edmund M. Buras, Jr., Washington, D.C., and Hermann J. Janssen, New Orleans, and John D. Tallant, Kenner, La., assignors to the United States of America as represented by the Secretary of Agriculture

No Drawing. Filed May 23, 1958, Ser. No. 737,456

1 Claim. (Cl. 8—132)

(Granted under Title 35, U.S. Code (1952), sec. 266)

A non-exclusive, irrevocable, royalty-free license in the invention herein described, throughout the world for all purposes of the United States Government, with the power to grant sublicenses for such purposes, is hereby granted to the Government of the United States of America.

This invention relates to a process for producing chemically modified cellulosic textiles with dimensional stability. More particularly this invention relates to a process of heat curing under stress fibrous cellulosic esters and ethers in the form of fiber, yarns, or fabrics.

The products prepared according to the process of this invention exhibit greatly reduced growth when subjected to cyclic loading. Growth, with specific reference to dimensional stability, may be defined simply as the amount of "bagginess" after repeated loading to less than the breaking strength of the material (approximately  $\frac{1}{3}$  the breaking strength).

Growth is defined above as the displacement of the tenth cycle hysteresis loop along the elongation axis (the upper limit of the loop being  $\frac{1}{3}$  of the breaking strength). Dimensional stability is a highly desirable characteristic in virtually every end use to which textile materials may be put. Dimensional stability is particularly desirable in the case of chemically modified cellulosic fibers and some obvious uses of dimensionally stabilized fabrics (i.e. fabrics that will resist growth or bagginess after being subjected to stress or tension) are in conveyor belts (paper drying belts), upholstery backings, articles of wearing apparel and the like. The combined effect of heat and tension as employed in the process of this invention does not materially impair the breaking strength of the textile material.

In general the process of this invention involves heating certain chemically modified cotton fibers in the form of yarns, or fabrics under tension. The operable temperature can vary from 100° C. to as high as 235° C., the upper practical limit being the onset of heat degradation in the material undergoing treatment. The time requirements for the treatments disclosed in this invention can vary from 30 seconds to as much as 8 minutes. The more extended heating periods are employed with the lower treating temperature. Tension (stress) in amounts approximating 50% of the original breaking strength of the materials undergoing treatment can be applied in the process. Tension approximating  $\frac{1}{3}$  of the breaking strength as measured under standard textile testing conditions of the material is preferred.

The heat treatment can be carried out as a continuous operation or as a batch operation. The treatments described in the specific examples which follow were carried out in a small, electrically heated and controlled cylindrical oven approximately 12 inches long. The effective heating chamber of the oven was approximately 9 inches in length. The cylindrical oven was positioned vertically with respect to its long axis. The particular oven em-

## 2

ployed was closed at both ends with Bakelite stoppers. Each stopper was provided with a narrow slot through its center to permit passage of the material undergoing treatment. The upper Bakelite stopper in the oven was drilled for insertion of the thermometer. The material undergoing treatment was supported outside and above the oven by means of clamps. The free end was threaded through first the upper oven stopper slot then down through the oven proper and out through the lower oven stopper slot. Through the slots and within the oven itself, the material undergoing treatment hung free. The lower emergent end of the material undergoing treatment was loaded with weights in order to provide tension. Treatment temperatures of 100° C., 200° C., and 235° C. were utilized along with various tensions up to 50% of the breaking strength of the original material. Treatment time varied from 30 seconds to 8 minutes.

The specific examples are simple batch type processing treatments but it will be recognized that a variety of known means can be employed to carry out the treatment in batch or continuous operation. In the specific examples and in the tabular data which follow we use the term "partially acetylated cotton" to describe cotton that has been treated with an acetylating agent (i.e. acetic anhydride) so as to esterify part but not all of the available hydroxyl groups on the cellulose. It is possible, by the use of catalysts and specific conditions, to replace as many as three hydroxyl groups per anhydroglucosidic unit of cellulose with acetyl groups (a degree of substitution of three). Partially acetylated cotton, we define as acetylated cotton which has a degree of substitution of from 0.5 to 2.0 substituted hydroxyl groups per anhydroglucosidic unit (acetyl content of from 12 to 35% based on the weight of the acetylated cotton). Fully acetylated cotton exhibits a degree of substitution of from 2.0 to 3.0 (acetyl content 35 to 45%).

The partially cyanoethylated cotton shown in Example 5 below, is a cotton with a degree of substitution of 1.1 to 1.3.

### EXAMPLE 1

Table I.—Properties of partially acetylated 8/5 yarns after treatment with heat and load for 30 seconds<sup>1</sup>

| 50                        | Conditions of treatment | Single strand breaking strength, lb. | Elongation-at-break, percent | Growth after 10 cycles, percent | Secant Modulus, lbs./100%<br>inches |
|---------------------------|-------------------------|--------------------------------------|------------------------------|---------------------------------|-------------------------------------|
|                           |                         |                                      |                              |                                 |                                     |
| Control (no heat or load) |                         | 12.9                                 | 9.9                          | 1.76                            | 130                                 |
| 100                       | 0                       | 12.4                                 | 8.8                          | 1.10                            | 141                                 |
| 100                       | 10                      | 13.6                                 | 11.4                         | 1.20                            | 119                                 |
| 100                       | 30                      | 13.4                                 | 8.3                          | 0.70                            | 161                                 |
| 100                       | 50                      | 12.3                                 | 6.2                          | .40                             | 198                                 |
| 150                       | 0                       | 13.9                                 | 10.2                         | 1.70                            | 136                                 |
| 150                       | 10                      | 13.8                                 | 7.8                          | 0.50                            | 177                                 |
| 150                       | 30                      | 12.0                                 | 5.2                          | .30                             | 231                                 |
| 150                       | 40                      | 10.0                                 | 4.2                          | .30                             | 238                                 |
| 200                       | 0                       | 14.0                                 | 11.4                         | 1.30                            | 123                                 |
| 200                       | 1                       | 13.4                                 | 8.2                          | 0.80                            | 163                                 |
| 200                       | 2.5                     | 13.7                                 | 8.3                          | .80                             | 165                                 |
| 200                       | 5                       | 11.8                                 | 6.8                          | .60                             | 174                                 |
| 200                       | 10                      | 12.9                                 | 5.0                          | .30                             | 258                                 |
| 200                       | 20                      | 12.5                                 | 4.9                          | .10                             | 255                                 |
| 235                       | 0                       | 12.8                                 | 9.3                          | 1.30                            | 138                                 |
| 235                       | 1                       | 11.5                                 | 8.2                          | 1.20                            | 140                                 |
| 235                       | 2.5                     | 12.0                                 | 7.3                          | 0.70                            | 164                                 |
| 235                       | 5                       | 11.7                                 | 6.6                          | .50                             | 177                                 |
| 235                       | 10                      | 12.5                                 | 6.2                          | .30                             | 202                                 |
| 235                       | 20                      | 10.9                                 | 4.5                          | .20                             | 242                                 |

<sup>1</sup> All samples were heated a total of 30 seconds with load and an additional 20 seconds without load (time necessary to apply and remove load). Samples with 0 load were heated 50 seconds.

Table II.—Properties of partially acetylated 8/5 yarn after treatment with heat and load for 1 minute<sup>1</sup>

| Conditions of treatment   |                                               | Single strand breaking strength, lb. | Elongation-at-break, percent | Growth after 10 cycles, percent | Secant Modulus, lbs./100% |
|---------------------------|-----------------------------------------------|--------------------------------------|------------------------------|---------------------------------|---------------------------|
| Temp., ° C.               | Load, percent of breaking strength of control |                                      |                              |                                 |                           |
| Control (no heat or load) |                                               | 12.9                                 | 9.9                          | 1.76                            | 130                       |
| 200                       | 0                                             | 13.2                                 | 9.5                          | 2.20                            | 139                       |
| 200                       | 20                                            | 13.4                                 | 5.0                          | 0.30                            | 268                       |
| 245                       | 0                                             | 12.2                                 | 9.1                          | 2.20                            | 134                       |
| 245                       | 20                                            | 12.3                                 | 3.8                          | 0.10                            | 324                       |

<sup>1</sup> All samples were heated a total of 1 minute with load and an additional 20 seconds without load (time necessary to apply and remove load). Samples with 0 load were heated for 1 minute and 20 seconds.

## EXAMPLE 2

Table I.—Effect of heat and load on properties of partially acetylated fabric

| Conditions of treatment                                 | Breaking strength, <sup>1</sup> lbs. | Elongation-at-break, percent | Growth after 10 cycles, percent | Secant Modulus, lbs./100% |
|---------------------------------------------------------|--------------------------------------|------------------------------|---------------------------------|---------------------------|
| Control (no heat or load)                               | 90.2                                 | 8.5                          | 1.84                            | 1,061                     |
| 4 min. heat (200° C.) (no load)                         | 89.2                                 | 7.0                          | 1.86                            | 1,274                     |
| 4 min. heat (200° C.) (2 min., 20% load 2 min., 0 load) | 87.0                                 | 3.1                          | 0.11                            | 2,806                     |

<sup>1</sup> Strip breaks on 96 threads.

## EXAMPLE 3

Table I.—Effect of heat and loading for 30 seconds on "growth" of fully acetylated yarn<sup>1</sup>

| Conditions of treatment |  | Load, percent of breaking strength of control | Growth (after 10 cycles), percent |
|-------------------------|--|-----------------------------------------------|-----------------------------------|
| Temp., ° C.             |  |                                               |                                   |
| Control                 |  |                                               | 11.5                              |
| No heat                 |  | 30                                            | 6.65                              |
| 100                     |  | 0                                             | 5.4                               |
| 100                     |  | 10                                            | 5.0                               |
| 100                     |  | 50                                            | 2.0                               |
| 150                     |  | 0                                             | 8.1                               |
| 150                     |  | 10                                            | 2.7                               |
| 150                     |  | 30                                            | 1.2                               |
| 200                     |  | 0                                             | 8.0                               |
| 200                     |  | 1                                             | 2.78                              |
| 200                     |  | 10                                            | 0.92                              |
| 235                     |  | 0                                             | 4.4                               |
| 235                     |  | 1                                             | 2.4                               |
| 235                     |  | 2.5                                           | 1.4                               |
| 235                     |  | 5                                             | 0.90                              |
| 235                     |  | 10                                            | .90                               |

<sup>1</sup> All samples were heated a total of 30 seconds with load and an additional 20 seconds without load (time necessary to apply and remove load). Samples with 0 load were heated 50 seconds.

Table II.—Effect of heat and load on properties of fully acetylated 10/3 yarn

| 5                                                              | Conditions of treatment | Single strand breaking lb. | Elongation-at-break, percent | Growth after 10 cycles, percent | Secant Modulus, lbs./100% |
|----------------------------------------------------------------|-------------------------|----------------------------|------------------------------|---------------------------------|---------------------------|
| Control                                                        |                         | 7.0                        | 23.8                         | 11.5                            | 29                        |
| 1 min., 20 sec. heat (200° C.)                                 |                         | 6.2                        | 22.8                         | 12.0                            | 27                        |
| 1 min. load (30%)                                              |                         | 6.7                        | 16.8                         | 6.65                            | 40                        |
| 1 min., 20 sec. heat (200° C.), 1 min. load (30%) <sup>1</sup> |                         | 8.0                        | 3.9                          | 0.40                            | 205                       |

<sup>1</sup> Heated 1 minute with load and an additional 20 seconds without load (time necessary to apply and remove load).

## EXAMPLE 4

Table I.—Effect of heat and load on properties of fully acetylated fabric

| 20                             | Conditions of treatment | Breaking strength, lb. | Elongation-at-break, percent | Growth after 10 cycles, percent | Secant Modulus, lbs./100% |
|--------------------------------|-------------------------|------------------------|------------------------------|---------------------------------|---------------------------|
| Control                        |                         | 152                    | 13.1                         | 5.08                            | 1,160                     |
| Heated 1.5 min., 200° C.       |                         | 152                    | 12.9                         | 5.00                            | 1,178                     |
| Loaded (20% breaking strength) |                         | 154                    | 11.8                         | 3.65                            | 1,305                     |

<sup>1</sup> Strip breaks on 100 threads.

## EXAMPLE 5

Table I.—Effect of heat and load on properties of partially cyanoethylated yarn<sup>1</sup>

| 30                              | Conditions of treatment | Breaking strength, g. | Elongation-at-break, percent | Growth after 10 cycles, percent |
|---------------------------------|-------------------------|-----------------------|------------------------------|---------------------------------|
| Control                         |                         | 1,318                 | 22.3                         | 11.6                            |
| 2 min., heat (200° C.) 20% load |                         | 1,337                 | 7.3                          | 0.78                            |

<sup>1</sup> 14/2 gray yarn 4.1 TM cyanoethylated in liquid phase.

## We claim:

A process comprising heating cyanoethylated cotton fibers having a degree of substitution of from 0.5 to 2.0 substituted hydroxyl groups per anhydroglucosidic unit at a temperature of from 100° to 235° C. for a period of from 30 seconds to 8 minutes while applying to the fibers tension in the amount of from  $\frac{1}{3}$  to  $\frac{1}{2}$  of the breaking strength of the partially cyanoethylated fibers to produce dimensionally stable partially cyanoethylated cotton fibers.

## References Cited in the file of this patent

## UNITED STATES PATENTS

|           |                  |               |
|-----------|------------------|---------------|
| 2,198,660 | Dreyfus          | Apr. 30, 1940 |
| 2,346,208 | Conaway          | Apr. 11, 1944 |
| 2,395,396 | Conaway          | Feb. 26, 1946 |
| 2,447,567 | Dreyfus          | Aug. 24, 1948 |
| 2,777,750 | Sprague et al.   | Jan. 15, 1957 |
| 2,862,785 | Finlayson et al. | Feb. 2, 1958  |
| 2,900,669 | Booth            | Aug. 25, 1959 |

## OTHER REFERENCES

Buras et al.: "New Textile Products From Cotton," Southern Utilization Research Branch, New Orleans, La., ARS-72-4, September 1956, pp. 1-24.